

April 30, 1963

B. F. FREEBERG

3,087,811

ALLOYS OF MERCURY

Filed Nov. 3, 1960

VARIATION OF THE FREEZING POINT WITH VARIATION OF  
THE THALLIUM CONCENTRATION



FIG. 1

VARIATION OF THE FREEZING POINT WITH VARIATION OF  
THE INDIUM CONCENTRATION



FIG. 2

INVENTOR.  
BENJAMIN F. FREEBERG  
BY *Norman Aon With*

ATTORNEY

## 1

3,087,811

## ALLOYS OF MERCURY

Benjamin F. Freeberg, Lombard, Ill., assignor to Vapor Corporation, a corporation of Delaware  
Filed Nov. 3, 1960, Ser. No. 66,979  
3 Claims. (Cl. 75—169)

The present invention relates to alloys and particularly to alloys for use in thermometers and thermostats of the liquid column type.

The alloy of the present invention embodies a three component amalgam of indium, thallium, and mercury which remains in a liquid state at extremely low temperatures and at temperatures below those of mercury alloys as heretofore known. The alloy is particularly suitable for use as the liquid medium in resistance devices, such as that disclosed in my U.S. Patent No. 2,906,981, and in thermostats such as is disclosed in Patent No. 2,596,825, issued to applicant and others. In this age of outer space exploration it is necessary to provide thermostatic devices capable of withstanding extremely low temperature which may be encountered in space or in low temperature environs wherein equipment may be stored.

The alloy herein disclosed has a freezing point of —82° F.

Accordingly, it is an object of my invention to provide a mercury composition which is susceptible to low freezing temperatures, retaining the liquid properties of mercury at such lower temperatures.

It is a further object of my invention to provide a eutectic mercury amalgam which may be used in connection with control equipment found in guided missiles, electronic signaling devices, outer space apparatus and aircraft generally, where extremely low temperatures may be encountered.

Another object of my invention is to provide an alloy for use in thermostats and thermometers which encounter temperatures of minus eighty degrees Fahrenheit (—80° F.) or lower.

It is a further object to provide a mercury composition which may be subjected to extremely low temperatures and which when brought to higher temperatures will retain its physical properties.

The characteristics of the alloy are demonstrated graphically wherein

FIGURE 1 depicts the results in freezing point variation with the variation of the thallium concentration; and

FIGURE 2 depicts the results in freezing point variation with variation of the indium concentration.

Mercury freezes at —40° F. and consequently its use in thermometers and in thermostats is limited to such sub-zero temperature range. In certain two component eutectic compounds, the freezing point may be lowered to —74° F. Such result is obtained with a mercury-thallium amalgam, wherein the thallium represents 8.75% by weight of the amalgam.

In the present invention, it has been discovered that the use of a three component system will further reduce the freezing point. Such a eutectic is comprised of indium, thallium, and mercury resulting in an amalgam which freezes at —82° F.

The composition of this alloy is:

|          | Percent |
|----------|---------|
| Indium   | 16.0    |
| Thallium | 14.3    |
| Mercury  | 69.7    |

## 2

The amalgam remains plastic at temperature as low as —86° F. This is of particular significance, in that breakage of the amalgam container will not occur when the container is brought into higher temperatures.

5 The amalgam herein disclosed has other desirable features. Its coefficient of expansion is greater than the coefficient of pure mercury. Further, the boiling point is elevated above that of pure mercury lending for greater versatility of use. The physical characteristics of this 10 alloy may be further described as follows:

|                                                           |                        |
|-----------------------------------------------------------|------------------------|
| A. Density, grams per cubic centimeter:                   |                        |
| At 80° F.                                                 | 11.723                 |
| At 0° F.                                                  | 11.797                 |
| At —50° F.                                                | 11.842                 |
| B. Thermal coefficient of cubical expansion per degree F. |                        |
| From 0° F. to +80° F.                                     | $78 \times 10^{-6}$    |
| From —50° F. to 0° F.                                     | $76 \times 10^{-6}$    |
| C. Specific resistance at 80° F., ohms per                |                        |
| cm. <sup>3</sup>                                          | $54.06 \times 10^{-6}$ |
| D. Dynamic viscosity, centipoises, at 68° F.              | 0.35990                |
| E. Specific heat, calories per gram                       | 0.356                  |

In the preparation of the amalgam, the proper amounts 25 of the indium and thallium are weighed and dissolved in a weighed amount of mercury. The resulting mixture is cooled to the eutectic temperature of —82° F. and filtered to remove compositions, if any, outside the eutectic range.

The proportions of the indium concentration may be 30 varied from 14.9% to 16.6% with corresponding variation of the thallium content within one degree of the prescribed eutectic temperature of —82° F. The results of such variation of the concentration of indium relative to thallium and vice versa in terms of freezing point

35 is shown in the attached graph. This data is depicted in the form of graphs shown in FIGURES 1 and 2 wherein the upper curve presents the temperature at which crystals starts to separate. The lower curve presents the temperature at which the solidification is complete.

40 The temperature corresponding to the areas between the curves embody a mixture of solid and liquid. The portion of the curves below the dotted line show the allowable composition if a freezing point of —81° F. is allowed. This is 1° F. above the eutectic freezing point.

Certain other variations in the proportions of the elements present in the alloy may be made without departing from the spirit of the invention or the scope of the appended claims.

What I claim is:

1. A mercury alloy consisting of from 13.1% to 15.5% thallium, 16.0% indium and from 68.5% to 70.9% mercury.
2. A mercury alloy consisting of from 14.3% to 16.7% indium, 14.3% thallium and from 69% to 74% mercury.
3. A mercury alloy consisting of 69.7% mercury, 16.0% indium and 14.3% thallium to provide a eutectic, the freezing point of which is —82° F.

## References Cited in the file of this patent

## UNITED STATES PATENTS

- 60 1,959,668 Gray ----- May 22, 1934  
2,906,981 Freeberg ----- Sept. 29, 1959